

## UNITED STATES PATENT OFFICE

RICHARD FRANCHOT, OF WASHINGTON, DISTRICT OF COLUMBIA, ASSIGNOR TO FERRO CHEMICALS, INC., OF WASHINGTON, DISTRICT OF COLUMBIA, A CORPORATION OF DELAWARE

## IRON SMELTING

No Drawing.

Application filed March 15, 1928. Serial No. 262,047.

This invention relates to iron smelting; and it comprises a process of smelting iron ores with solid carbonaceous fuels and pre-heated air in a blast furnace provided with 5 hot gas outlets for the diversion of gas and saline vapors wherein the temperature of the air blast is much lower than in current practice, the burden of ore is nevertheless substantially larger; the slag is less basic or 10 more siliceous, while the gas passing out the furnace top is substantially spent; all as more fully hereinafter set forth and as claimed.

Exactly one hundred years ago the hot blast was patented by Neilson in Great Britain. The use of blast heat effects a saving in the coke required to smelt iron amounting to as much as 75 per cent of that needed with cold blast. It also materially increases 20 furnace capacity. The development of later day practice has been toward the use of higher and higher blast temperatures until 1600° F. or higher is not uncommon. Other things being equal, the greater the blast heat 25 the better is the fuel economy; that is to say, the ratio of ore to coke may be increased with increase of blast temperature. However, much irregularity is found in the rate of efficiency increase with increase of blast heat, 30 the returns in fuel saving with the higher blast temperatures being substantially diminished. The functional variation is not linear. The use of great blast heats is often attended with operating troubles; there being 35 sometimes no economy in the highest blast temperatures.

In prior patents, notably 1,466,644 of Aug. 28, 1923 and 1,555,784 of Sept. 29, 1925, are described methods and means of improving 40 the fuel economy of the blast furnace process wherein the furnace is provided with outlets for hot gases carrying out of the hot zone alkali cyanid and other saline matter in vapor form, thereby preventing or limiting the accumulation in the furnace of such volatile matter, and wherein the rate of driving and the burden of ore charged with the coke are substantially increased over rates of driving and burden ratios used without hot gas and saline 45 vapor diversion, the blast heat being varied in

inverse proportion with the rate of hot gas diversion, and the use of the highest possible blast temperatures being recommended. In the practice of these inventions the benefit of high blast temperatures is more marked 55 than in the prior art and the use of extreme blast heats and high rates of driving, with consequent economy much better than theretofore considered possible, has become practicable. In other words, there has been less 60 diminishment of return from blast temperatures ranging up to above 1600° F. In these inventions the chemical activity of the air nitrogen is controlled by limiting alkali accumulation in the furnace with its consequent 65 cyanid vapor formation and associated heat absorption in the hearth or combustion zone.

I have discovered that, with a diversion from the furnace of hot gases and saline vapors in amounts and at temperatures sufficient 70 to prevent undue accumulation of alkalies in the furnace and thus to hold a relatively low concentration of alkali (cyanid) vapor in the hearth gases, it is possible to run with a moderate blast temperature and at the same time 75 to charge with the coke a burden of ore larger than has even been done with the greatest blast heats. I find that a blast temperature around 900° F. results in greatly improved fuel economy and makes possible a fast rate 80 of driving without necessitating an undue diversion of gas for heating the blast. With blast temperatures of 900° F. and below, vaporization of slag is relatively small. A blast temperature between 700° and 900° F. 85 is usually suited to a diversion from the hot zone of between 20 and 25 per cent of the gases formed in the hearth. A higher blast temperature may require a greater rate of diversion in order to provide fuel for heating 90 the blast. With adequate alkali or cyanid vapor outlet, a limitation of the blast heat further limits the chemical activity of the air nitrogen not only by lowering the combustion temperature but also by limiting the expulsion of alkali vapor from the slag, the latter limitation itself increasing the availability of the combustion heat for maintaining high hearth temperatures. A further 95 effect of the lower blast heat is that of limit- 100

ing slag vaporization with its attendant heat absorption. And when, in turn, the burden of ore is adjusted to the increase of available heat, then, as I have found, the furnace works smoothly and much more uniformly than heretofore. Even with quite low blast temperatures it is possible to make the burden great enough to cause substantially complete utilization of the latent energy of the gas 5 put through the shaft, as evidenced by a top gas composition showing CO<sub>2</sub> ratios closely approaching 100 per cent, that is, with practically all CO converted to CO<sub>2</sub>.

In the present invention fuel economy is 10 improved over prior practice by decreasing the blast heat while increasing the ore burden. The blast heat should be in direct relation with the rate of hot gas diversion the blast temperature being raised or lowered as the 15 proportion of gas diverted is made greater or smaller. With a diversion rate about the equivalent of 25 per cent of the gases formed by the air blast the blast temperature may still be kept below 900° F. If desired, the 20 temperature of the blast may be that of the atmosphere, it being practicable to work with cold blast when a relatively large diversion of fuel gas is desired for the sake of the gas. However, it is better practice to divert a 25 smaller amount of gas and to work with a moderate blast heat, proportioning the blast heat in direct ratio with the amount of gas diverted. The amount of gas to be diverted depends somewhat upon the alkali content 30 (K<sub>2</sub>O and Na<sub>2</sub>O) of the material smelted; ore and coke of relatively higher alkali content requiring a greater diversion of gas than others in order to prevent undue accumulation 35 of alkali in the furnace. Ordinarily, for example, Southern ores, by reason of their higher potash content, require a greater proportion of the gas to be diverted than do the Lake ores; this difference, however, being modified in some instances by the greater 40 amounts of gangue in the Southern ores, requiring more heat for fluxing. In general, a diversion of the equivalent of about 25 per cent of the air gas at a temperature around 45 2200° F. works well with a blast temperature from 800 to 900° F. In adjusting these 50 two factors in correlation for purposes of regulation the blast heat is lowered or raised as the diversion of hot gas is decreased or increased. In some cases good fuel economy is 55 obtainable with blast temperatures around 500° to 600° F. but in general a better balance is secured with a heat of 800° to 900° F. The blast temperature is conveniently regulated by mixing unheated air by well known means 60 with air heated to temperatures above the one desired. While the blast temperature is thus limited the burden is made relatively large. Even with moderate blast heats and with a 65 20 to 25 per cent hot gas diversion, the ore burden, the ratio of ore to coke, is made great-

er than has ever been found practicable with the greatest blast heat without hot gas diversion, greater indeed than has hitherto been generally considered theoretically possible. The burden should be at least great enough 70 to prevent solution loss, that is, the gasification of coke carbon otherwise than by air. The amount of ore charged with the coke may be that sufficient to convert to CO<sub>2</sub> all the CO formed by the air oxygen less the amount of 75 CO diverted in hot gas; this CO<sub>2</sub> formation being effected through direct oxidation by the oxids of the charge aided by the breaking up of 2CO into C and CO<sub>2</sub>, the latter action being promoted by the extension of the 80 zone of temperature suitable thereto which results from the diversion of hot gas and the adjustment of the ore burden. In addition, a third positive beneficial step is possible, namely that of putting into the charge an 85 amount of basic flux, limestone or dolomite, substantially less, relative to the silica and alumina contained in the ore and coke than is usually charged, this step having the effect 90 of making the slag less basic or more siliceous 95 than heretofore. This is made permissible by the greater production of iron and slag per unit of coke and thus by the greater slag volume per unit of sulfur input, the latter being usually for the most part a matter of the sulfur in the coke. To adequately eliminate sulfur from the iron the proportion by weight of lime and magnesia together to silica and alumina together may be, with coke sulfur 100 well over 1 per cent, substantially less than 105 the usual 1 to 1. This proportion of bases may average less than 0.8 to 1 and it may be considerably lower. The step of lowering the ratio of lime and magnesia to silica and alumina is in itself beneficial by way of decreasing 110 the expulsion of alkali vapor (potash and soda) from the slag, thereby lessening alkali accumulation and vaporization with cyanid formation, hence by way of making more heat available to the hearth for strictly smelting work and thus of permitting a further increase of burden. Decreasing the bases is 115 beneficial also in making it easier to put silicon into the metal, when desired.

The three steps: (1) lowering the blast temperature, (2) increasing the ore burden, and (3) lessening the slag basicity, are cumulatively and interdependently beneficial. Improvement upon prior inventions is secured by way of reducing the requirement of gas to 120 be diverted; less fuel and smaller plant capacity being now needed for heating the blast. There is a further advantage in being able 125 always to have a substantial reserve of blast heat. Furthermore, as a result of lessened nitrogen activity associated with smaller blast heats and larger burdens, the metal produced contains less nitrogen and is of superior quality. The process controls the rejection of unutilized energy from the furnace and at the 130

same time delivers the rejected energy in the form of a hot rich gas which is more efficient as a fuel than the blast furnace gas ordinarily produced.

As an example embodying the principles of this invention may be taken the smelting of hematite ore having a natural content of 52 per cent iron and 11 per cent silica and alumina with coke containing as charged 85 per cent fixed carbon, 1.1 per cent sulfur and 12 per cent ash consisting mainly of silica and alumina; the flux used being a 60:40 mixture of limestone and dolomite containing as available bases 44 per cent lime and 9 per cent magnesia. To make foundry iron of such materials in a furnace of 24,000 cubic feet working volume taking 43,000 to 47,000 cubic feet of air per minute (60° F. and one atmosphere pressure), the furnace being provided near the top of the bosh with four gas outlets about 4 feet in diameter throttled down to maintain adequate furnace pressure and delivering into a valve controlled gas conduit, the amount of gas diverted should be about 13,000 cubic feet of free gas per minute (atmospheric temperature and pressure) having as it leaves the furnace a temperature of 2200° F., the blast temperature is best kept between 700° and 800° F. and the ore burden charged with the coke can then be in a ratio of 2.9 to 1, with stone mixture added to the extent of 18 per cent of the weight of ore. The rounds charged may be the equivalent of 13,000 lbs. coke, 37,700 lbs. ore, 4,070 lbs. limestone and 2710 lbs. dolomite. With the described rate of blowing, hot gas diversion, blast heat and burden ratio the furnace can produce daily over 780 tons of foundry iron averaging 2.5 per cent silicon and 0.025 per cent sulfur with a consumption of about 1400 lbs. coke per ton, a pig iron yield of over 55 per cent on the ore and a slag volume of about 41 per cent of the weight of pig or 320 tons per day, using 760 lbs. stone per ton of iron; the slag analyzing 56 per cent silica and alumina to 43 per cent lime and magnesia and 1.4 per cent sulfur (the diverted hot gas carrying considerable sulfur out of the furnace); the gas diverted being some 24,000 cubic feet per ton of iron and having a calorific value between 120 and 130 B. t. u. per cubic foot, with upwards of 40 B. t. u. of sensible heat in addition.

The above exemplified production is at a rate of about 2 pounds iron with its accompanying slag and gas per pound of carbon burning with air. It may be noted that the oxygen removed from the ore in reduction of 2 lbs. of this iron is the amount used in oxidizing 0.64 lb. carbon from CO to CO<sub>2</sub>. Hence, with a diversion from the top of the bosh of 13,000 cubic feet of gas per minute, which is somewhat less than 25 per cent of the gas produced by the air blown, the burden of ore gives up to the gases an amount of oxygen sufficient to convert to CO<sub>2</sub> 64 per cent out of the 75 per

cent of the CO formed by the air which is caused to flow up through the shaft, or some 85 per cent of the undiverted CO. It is also to be noted that the blast temperature, 750° F., makes the heat generated in CO formation by the air oxygen plus the blast heat 5420 B. t. u. per pound carbon, of which some 30 per cent (about 800 B. t. u. per pound pig) is available in the hearth at 2700° F. A 25 per cent loss in water cooling and radiation, 1350 B. t. u. per pound carbon, leaves 4,000 B. t. u. effective. Of this, 950 B. t. u. being taken out as sensible heat of the gas diverted at 2200° F., the remaining heat 3050 B. t. u., is sufficient to supply the 2560 B. t. u. absorbed in heating the metal and slag and decarbonating the stone (oxidation of CO to CO<sub>2</sub> by the oxids of the ore being exothermic). The unused heat as generated by the air (490 B. t. u.), together with the latent heat of carbon deposition in 12 per cent of the CO formed by air oxygen and unused in reduction (350 B. t. u.), constitute a surplus of 840 B. t. u. per pound carbon burning with air. This surplus is available for drying the charge and heating the top gases to a moderate temperature, 200° to 250° F. Any temporary deficiency of heat can be supplied by increasing the blast volume without burning any more coke, the rate of heat generation being thus increased both by increasing the combustion of carbon in the hearth and by increasing the deposition of carbon in the shaft. The carbon deposited (equal to about 6 per cent of that burning with air) may be nearly or quite sufficient to supply that dissolved in the metal, in fact, it is possible to have the air burn more carbon than is charged as coke. In the described process substantially all the CO passed up the shaft may be converted to CO<sub>2</sub>, partly in direct reduction of iron oxid, partly in carbon deposition. The top gas is thus completely spent. The hot gas diverted from the bosh contains in sensible heat and combustible components (CO and H<sub>2</sub>) somewhat more than 20 per cent of the calorific energy of the coke fed to the furnace; the blast heat being about 8 per cent of the coke energy. In efficient recuperators and power plants the diverted hot gas suffices for heating and blowing the air blast. A part of whatever alkali that may be contained in the ore and coke is recoverable as cyanid from the diverted gas, using the air as a cooling agent. Normally a recovery of at least a ton of potassium cyanid per day is possible.

The chief benefit to be derived from the present invention is that of improved economy in iron smelting. Compared with current practice without hot gas diversion but with blast temperatures above 1200° F., it is now possible with blast temperatures below 900° F. to increase furnace production by 20 to 30 per cent without increase of blast volume and with a substantial decrease of

daily coke consumption. Using coke the metallurgy of the furnace may be made more efficient than the best charcoal practice has been; the quality of the produced iron being for many purposes improved.

In further contrast to prior practice using very hot air, with or without diversion of hot gas, the present invention lends itself to ready control of the gas producing function of the blast furnace. The new process may confine the rejection of latent energy by the furnace to the rich gas diverted near the bottom and when an increased production of fuel gas is desired, all that is necessary is to decrease the amount of ore charged with the coke and to increase the diversion of gas.

I claim:

1. In smelting iron ores with solid carbonaceous fuels and preheated air in a blast furnace to produce iron alloys, fuel gas and slag, the process which comprises diverting a limited amount of hot gases and saline vapors from the hot zone of the furnace and introducing the air blast at a temperature below 900° F.

2. In smelting iron ores with solid carbonaceous fuels and preheated air in a blast furnace to produce iron alloys, fuel gas and slag, the process which comprises diverting a limited amount of hot gases and saline vapors from the hot zone of the furnace, introducing the air blast at a temperature below 900° F., and charging with the fuel an amount of ore and flux sufficient to convert to  $\text{CO}_2$  substantially all the CO in the undiverted gases.

3. In smelting iron ores with solid carbonaceous fuels and preheated air in a blast furnace to produce iron alloys, fuel gas and slag, the process which comprises diverting a limited amount of hot gases and saline vapors from the hot zone of the furnace, introducing the air blast at a temperature below 900° F., charging with the fuel an amount of ore and flux sufficient to convert to  $\text{CO}_2$  substantially all the CO in the undiverted gases, and maintaining in the slag a proportion by weight of less than eight parts of lime and magnesia taken together to ten parts of silica and alumina taken together.

4. In smelting iron ores with solid carbonaceous fuels and preheated air in a blast furnace to produce iron alloys, fuel gas and slag, the process which comprises diverting a limited amount of hot gases and saline vapors from the hot zone of the furnace, introducing the air blast at a temperature below 900° F., and maintaining in the slag a proportion by weight of less than eight parts of lime and magnesia taken together to ten parts of silica and alumina taken together.

5. The process of improving fuel economy in smelting alkaliferous iron ores with coke and preheated air in a blast furnace to produce iron alloys, slag and fuel gas which com-

prises diverting hot gas and alkali vapors from the hot zone of the furnace, lowering the blast temperature and increasing the ratio of ore burden to coke.

6. The process of improving fuel economy in smelting alkaliferous iron ores with coke and preheated air in a blast furnace to produce iron alloys, slag and fuel gas which comprises diverting hot gas and alkali vapors from the hot zone of the furnace, lowering the blast temperature, increasing the ratio of ore burden to coke, and lessening the slag basicity.

7. In the operation of a blast furnace for the production of iron alloys and slag, burning coke with a preheated air blast to generate heat in the furnace hearth, the process which comprises diverting a limited amount of hot gases from the hot zone of the furnace and adjusting the blast temperature in direct proportion with the amount of gases so diverted, the blast temperature being raised as the rate of hot gas diversion is increased and lowered as the diversion rate is decreased.

8. In smelting iron ores with carbonaceous fuels and preheated air in a blast furnace, the process which comprises diverting a limited amount of gas from the furnace at a temperature around 2200° F., transferring heat from the diverted gas to the air blast and lowering or raising the temperature of the blast respectively by decreasing or increasing the rate of diversion of hot gas from the furnace, thus compensating the increase or decrease of diverted energy by increase or decrease of blast heat.

9. In the smelting of iron ores with coke and preheated air in a blast furnace with diversion of hot fuel gas from the hot zone of the furnace, the method of regulating the furnace operation which comprises adjusting the amount of fuel gas diverted in direct relation with the blast temperature, said diversion being increased with rise of blast temperature or decreased with drop in said temperature.

10. In operating a blast furnace for smelting iron ores with coke and preheated air while withholding from the shaft some of the hot gases produced in the hearth, the process which comprises keeping the blast temperature below 900° F. and adjusting the amount of ore charged with the coke to the amount of gas put through the shaft, charging sufficient ore to utilize substantially all the energy of the gas put through the shaft, and thus causing the gas leaving the top of the furnace to be nearly spent, that is to possess substantially no latent calorific energy.

In testimony whereof, I have hereunto affixed my signature.

RICHARD FRANCHOT.